

W. A. HALL.

PROCESS OF OBTAINING SULFUR FROM SULFIDS.

APPLICATION FILED JUNE 13, 1913.

1,083,251.

Patented Dec. 30, 1913.



FIG. 1.



FIG. 2.

Witnesses,

L. N. Gillis

A. B. Foster

William A. Hall <sup>Inventor:</sup>

John T. Albee <sup>Attorneys:</sup>

# UNITED STATES PATENT OFFICE.

WILLIAM A. HALL, OF NEW YORK, N. Y.

## PROCESS OF OBTAINING SULFUR FROM SULFIDS.

1,083,251.

Specification of Letters Patent. Patented Dec. 30, 1913.

Application filed June 13, 1913. Serial No. 773,456.

*To all whom it may concern:*

Be it known that I, WILLIAM A. HALL, a citizen of the United States, residing at New York, in the county of New York and State of New York, have invented or discovered certain new and useful Improvements in Processes of Obtaining Sulfur from Sulfids, of which the following is a specification, reference being had therein to the accompanying drawings.

In my copending application Serial No. 725,024, I have described and claimed a process of obtaining sulfur from metal sulfids such for example as pyrites, pyrrhotite and the like, by heating the same by the action of a reducing flame to a temperature maintained high enough to distil the sulfur, (between 700 and 900° C.), while introducing a small amount of steam into contact with said sulfids, and also while agitating the sulfid ore under treatment. This treatment is preferably carried out in a mechanical, reverberatory, multiple shelf furnace, and the conditions in each of the reaction zones may be about the same.

The present invention relates to an improvement on said process, in which ore is treated preferably in a furnace of the same general structure, but in which the conditions maintained in the several compartments differ from each other.

In carrying out the process I may use a furnace constructed as shown in the annexed drawings, in which—

Figure 1 shows a vertical section of the furnace, and Fig. 2 shows a horizontal section, on the line A—A of Fig. 1.

In operating in accordance with the present invention the metal sulfid, which may be pyrites or pyrrhotite or other metal sulfids is introduced from the hopper 1, located over the top of the furnace into the first compartment 2, and thence passes through the opening 3, into compartment 4, and so on downwardly to the several compartments 5, 6, 7, 8 and 9 of the furnace until it reaches the outlet 10 where it is discharged from the furnace.

In each of the compartments the sulfid is subjected to the action of a flame introduced by suitable burners 11, while steam is introduced into the upper compartments through suitable pipes 12, and also may be intro-

duced in smaller amounts into the lower compartments if desired, or may be omitted from these lower compartments.

On the upper shelves I maintain a very highly reducing flame, together with a considerable amount of steam, in order to produce the largest amount of  $H_2S$  possible, and in each successive zone of the furnace the flame is maintained less reducing and a smaller amount of steam is admitted, until the sulfid reaches the lowermost part 9, where it is treated with a flame which may be oxidizing and with a very small amount of steam, or none at all.

In the several compartments of the furnace are mounted any suitable rabbles 14, carried by the hollow shaft 15, which shaft may be air cooled if desired, and the rabbles may be air cooled or water cooled if desired. The temperature in the reaction zone will in this manner be successively higher in each successive compartment, which temperature will preferably be about 700° C. in the uppermost compartments, while in the lower compartments the temperature is maintained considerably above 700° C., and may be up to 900° C. in the last compartment. As a result of this treatment very large amounts of  $H_2S$  are formed in the uppermost compartments, also a quantity of free sulfur is distilled, while in the compartment near the middle a very large amount of free sulfur is distilled while only a comparatively small amount of  $H_2S$  is produced or even no  $H_2S$  at all, and in the lowermost compartments considerable  $SO_2$  will also be formed if the flame is oxidizing.

Instead of allowing the gases and vapors to pass principally upwardly through the furnace as in my prior application above referred to, I find it preferable to withdraw from each of the compartments the major portion of the gases into a suitable stand pipe or stack 16, from whence they are carried to suitable washing appliances for the recovery of the sulfur therefrom.

The principal reason for withdrawing as much as possible of the gases from each compartment is that these gases do not support combustion, but serve to dilute the active atmosphere in each of the compartments, especially the uppermost ones if allowed to pass upwardly, from shelf to shelf, as in my

- prior application above referred to, thus interfering with the combustion of the reducing flames on the upper shelves more or less.
- 5 The flame in the lowermost compartment, may be neutral, or even slightly oxidizing, according to the circumstances present, the kind of ore treated and the amount of sulfur therein.
- 10 In each of the flues 17, which connect the several compartments with the stack 16, I preferably provide a suitable damper, in order to control the flow of the gases through these several flues, in such a manner that 15 substantially all the gases produced in each compartment travel directly into the stack 16, and not into the next higher compartment of the furnace, as in my prior application above referred to.
- 20 In order to avoid too much false air being admitted into the furnace, I preferably maintain a very slight pressure (above atmospheric) within the furnace, although if the furnace be reasonably tight, this precaution 25 may not be necessary. The gases may be carried off from the stack 16 to the washers by means of any suitable pump located between said stack 16 and the washers, or located beyond the washers.
- 30 The removal of the sulfur content is much more rapid from the fresh ore than from the partially decomposed ore, and I find that the evolution of  $H_2S$  and free sulfur vapor in the uppermost compartments is 35 very rapid.
- It will be noted that in this respect the present process differs from the process of any copending application in that in said application I seek to produce only a distillation of free sulfur and to keep down the formation of  $H_2S$  as much as possible, while in the present process I seek to produce as much  $H_2S$  as possible, on all the upper shelves where I am distilling free sulfur, 40 in order to utilize this  $H_2S$  to combine with the  $SO_2$  produced on the lower shelves, and which lower shelves I use to a considerable extent, the same as in the ordinary ore roasting process, and I find by repeated tests that 45 the  $SO_2$  produced in the latter part of the operation is very weak, and can all be de-oxidized by the large amount of  $H_2S$  produced in the earlier stages of the process.
- Accordingly I can run the upper shelves for 50 the distillation of sulfur and the generation of  $H_2S$  and the lower shelves as an oxidizing or ore roasting operation, thereby generating  $SO_2$  and mingling all the fumes together in one common stand pipe or flue. If de- 55 sired I may also use air alone (without any gas flames) on the lower shelves, although better results may be obtained by using some gas along with the air.

The method of producing  $H_2S$  and the

furnace structure, are not claimed herein, 65 since these form the subject matter of my copending applications 725,026, and 725,023, respectively, both filed Oct. 10, 1912.

What I claim is:—

1. A process of separating sulfur from 70 sulfid ores, which comprises exposing said ores, in each of a plurality of successive steps, to the simultaneous action of a flame and of steam, the quality of the flame, as regards reducing power, being different in 75 the different steps.

2. A process of separating sulfur from sulfid ores, which comprises exposing said ore, in each of a plurality of successive steps, to the simultaneous action of a flame and of 80 steam, and quality of the flame, as regards reducing power, and the relative amount of steam employed, being different in the different steps.

3. A process of separating sulfur from 85 sulfid ores which comprises exposing said ores in each of a plurality of successive steps, to the simultaneous action of a flame and of steam, the reducing power of the flame being less in the later steps, than in 90 the earlier steps.

4. A process of separating sulfur from a sulfid ore which comprises subjecting said ore to a highly reducing flame and to a large 95 amount of steam, then exposing said ore to a flame of less reducing power, and to a smaller amount of steam, and then exposing said ore to an oxidizing flame in the absence of material quantities of steam.

5. A process of separating sulfur from 100 sulfid ores which comprises exposing said ores, in each of a plurality of successive steps, to the simultaneous action of a flame and of steam, the quality of the flame, as regards reducing power, being different in 105 the different steps, and agitating said ore during said treatment.

6. A process of separating sulfur from sulfid ore which comprises subjecting said ore to a highly reducing flame and to a large 110 amount of steam, then exposing said ore to a flame of less reducing power, and to a smaller amount of steam, and then exposing said ore to an oxidizing flame in the absence of material quantities of steam, and agitating the ore during each of said flame treatments.

7. A process of separating sulfur from sulfid ores, which comprises subjecting said ore, in a plurality of steps to the action of 120 steam in different amounts, and to the action of flames of different reducing power, separately drawing off the gases and vapors evolved in said separate steps, and then combining said gases to obtain sulfur therefrom.

8. A process of separating sulfur from ores which comprises subjecting said ore to

the action of a reducing flame and of steam, and thereafter subjecting said ore, while in a heated state to oxidation.

9. A process of separating sulfur from ores which comprises subjecting said ore to the action of a reducing flame and of steam, and thereafter subjecting said ore, while in a heated state to oxidation, and separately drawing off the gases and vapors produced

in each of said steps, and mingling said gases and vapors together for obtaining free sulfur.

In testimony whereof I have affixed my signature in presence of two witnesses.

WILLIAM A. HALL.

Witnesses:

A. M. PERKINS,  
M. R. MCKAY.